

Feb. 13, 1940.

G. C. GAUT ET AL  
ELECTROLYTIC CELL

2,190,285

Filed Feb. 28, 1938



Fig. 1



Fig. 2



Fig. 3



Fig. 4



Geoffrey Charles Gaut  
David John Pritchard Phillips  
INVENTORS

BY

*John Pritchard*

ATTORNEY

## UNITED STATES PATENT OFFICE

2,190,285

## ELECTROLYTIC CELL

Geoffrey Charles Gaut, Romford, and David John Pritchard Phillips, Croydon, England, assignors to P. R. Mallory & Co., Inc., Indianapolis, Ind., a corporation of Delaware

Application February 28, 1938, Serial No. 193,191  
In Great Britain October 19, 1937

4 Claims. (Cl. 175—315)

This invention relates to improvements in electrolytic condensers and like cells.

An object of the invention is to provide improved conductive spacers for use between electrodes of devices of this character.

Other objects of the invention will be apparent from the following description taken in connection with the appended claims.

The present invention comprises the combination of elements, methods of manufacture, and the product thereof brought out and exemplified in the disclosure hereinafter set forth, the scope of the invention being indicated in the appended claims.

15 While a preferred embodiment of the invention is described herein, it is contemplated that considerable variation may be made in the method of procedure and the combination of elements without departing from the spirit of the invention.

In the drawing:

Figure 1 illustrates a step in making the spacers of the present invention;

Figure 2 shows another step in producing one embodiment of the invention;

Figure 3 illustrates a condenser assembly embodying the spacers of the present invention; and

Figure 4 shows a completed condenser.

According to one feature of this invention a dry spacer which requires no impregnation, may if desired be manufactured independently of any other step in the process of manufacture of the cell, may be readily reeled or otherwise handled mechanically, and may be stored without difficulty, is manufactured by forming a solution of a suitable cellulose derivative, adding thereto at least one ionogen and at least one high-boiling liquid which is not a solvent for the cellulose derivative, and casting or otherwise treating the resulting mixture to produce a sheet, film or the like of the requisite dimensions; the solvent is wholly or partially removed at this last stage.

According to another feature of the invention a spacer is prepared by the steps specified in the preceding paragraph with the exception that the ionogen and high-boiling liquid are partially or wholly combined, prior to their addition to the solution of cellulose derivatives, to form a reaction product.

50 In either case the mixture is conveniently, but not essentially, cast as a film in continuous lengths on a travelling bend or rotating drum, the surface of which must be such as to avoid detrimental effects on the mixture; the dry film is stripped therefrom by any suitable means such as those known in the art of casting cellulose-derivative films and the casting machine may be similar in all respects to those employed in that art. Alternatively the mixture may be cast on 55 one of the cell electrodes, which is preferably

previously etched, or on a band of non-absorbent gauze, e. g. sized gauze, which acts solely as a mechanical stiffener and is not impregnated by the mixture.

The term "suitable cellulose derivative" is to be understood to exclude derivatives which product corrosion of the electrodes upon decomposition, such as nitrocellulose, and those which contain free sulphates or chlorides. The preferred derivative is cellulose acetate but ethyl cellulose and cellulose aceto-butyrate may be mentioned as suitable alternatives. The solvent is preferably a low-boiling solvent such as acetone, methyl acetate or ethyl formate but a solvent of higher boiling point than these, such as ethylene glycol diacetate, may be used provided that it is one that evaporates more quickly from the mixture during casting than the high-boiling liquid; two or more of these solvents may, of course, be used simultaneously.

20 The ionogen may be one or more of the acids used in the formation of conductive compositions for electrolytic condensers, such as citric or boric acid, and/or one or more stable salts thereof, preferably ammonium salts.

25 Ethylene glycol, diethylene glycol, triethylene glycol and glycerine are suitable high-boiling liquids.

The spacer produced by this invention consists of a non-tacky non-homogeneous (porous) 30 matrix of cellulose derivative carrying an electrolyte.

If desired the mixture may also include an ingredient, preferably an organic borate compound such as amyl borate, to give a plastic product, and/or a filler such as shellac or colophony resin.

In some cases the mixture may be cast hot but it is usually desirable to arrange matters so that it can be cast cold, the advantage of this being that subsequent detrimental absorption of water is reduced or avoided.

Example I.—A dope is prepared by dissolving 450 grams of cellulose acetate in 3½ litres of acetone and the following mixed ingredients are then added to the dope:

|                 | Grams |
|-----------------|-------|
| Amyl borate     | 350   |
| Ethylene glycol | 750   |
| Glycerine       | 150   |
| Citric acid     | 80    |
| Ammonium borate | 250   |

The mixing of these ingredients may be accelerated if desired by heating to a temperature of 55 75 to 80° C. They are added slowly to the dope with vigorous stirring by stirring means which are inert as regards the mixture, i. e. cause no reaction and do not dissolve. Rods of glass, aluminum or stainless steel are suitable.

The mixture thus obtained is preferably filtered and de-aerated either by heating, e. g., in a container surrounded by hot water, or by suction in order to avoid the formation of bubbles during casting. The mixture is cast hot, e. g., at a temperature of 70 to 80° C. for a linear casting band speed of 2 ft. per minute, the band being preferably of aluminum or stainless steel. If a band of nickel, copper or other material having detrimental effects on the mixture is required to be used it must be provided with a protective layer, e. g. of benzyl cellulose. The greater part of the acetone is given up by the mixture at this stage. The thickness of the film may be from two to three thousandths of an inch.

An operating economy may be obtained by arranging to recover the acetone given off in the casting operation.

20 The cast mixture must be used quickly if atmospheric conditions are such as to offer the risk of undue absorption of water.

Example II.—A composition as specified in the above example is used with the addition of 25 320 grs. of distilled water, the water being added to the five ingredients tabulated prior to their incorporation in the cellulose acetate dope. This modified mixture can be cast cold, giving a product which is less prone to the absorption 30 of atmospheric moisture than a mixture which is cast hot. Filtering and de-aerating of the mixture may be effected prior to casting.

Example III.—A mixture is prepared as in Example I except that 100 grs. of shellac are added 35 to the cellulose acetate solution before the addition of the remaining five ingredients.

Example IV.—A mixture is prepared from the following ingredients:

|                          |        |     |
|--------------------------|--------|-----|
| 40 (1) Cellulose acetate | grams  | 450 |
| (2) Amyl borate          | do     | 350 |
| (3) Diethylene glycol    | do     | 750 |
| (4) Glycerine            | do     | 150 |
| (5) Ammonium borate      | do     | 600 |
| 45 (6) Ethylene glycol   | do     | 450 |
| (7) Citric acid          | do     | 250 |
| (8) Distilled water      | do     | 300 |
| (9) Acetone              | litres | 6   |

50 Ingredients 3, 4, 5 and 6 are first mixed together and heated at 135° C. for twelve hours to give a reaction product. This product has added to it ingredient 2 with vigorous stirring and then the solution obtained by mixing ingredients 7 and 8 is added. Finally the resulting mixture 55 while still hot (at 75 to 80° C.) is added to the dope formed by mixing ingredients 1 and 9. The final mixture is cast hot as described with reference to Example I.

60 Referring to the drawing Figure 1 shows the step in the manufacture of the spacers wherein band 10 is passed through one of the mixtures 11 heretofore described so as to receive a film 12 of the mixture which is allowed to dry thereon. The band 10 may be a metal band used merely 65 for the purpose of casting the film 12 in which case the film is subsequently stripped off, as by blade 13, as shown in Figure 2, and rolled up into a roll 14 for subsequent use.

70 In other cases band 10 may be the intended condenser electrode itself, preferably etched, in which case the film 12 is allowed to remain as a coating on the electrode in the finished condenser. In still other cases the band 10 may be a strip of sized cloth, as described, which 75 serves as a base for the completed spacer.

Figure 3 shows a condenser assembly comprising spacers 12 of the present invention assembled with electrodes 15 and 16 of film forming metal, at least one of which is film-formed, the electrodes being provided with tabs 17 and 18, 5 respectively, for terminal connections.

Figure 4 shows a complete condenser in section, comprising the assembly of Figure 3 rolled up into a roll 19 and enclosed in a container 20 sealed by an insulating cap 21 and having 10 terminals 22 and 23 connected to the tabs 17 and 18.

While the present invention, as to its objects and advantages has been described herein as carried out in specific embodiments thereof, it 15 is not desired to be limited thereby but it is intended to cover the invention broadly within the spirit and scope of the appended claims.

What is claimed is:

1. A film-maintaining spacer for dry electrolytic condensers comprising a non-tacky, non-homogeneous, porous matrix of cellulose derivative selected from the group consisting of cellulose acetate, ethyl cellulose and cellulose aceto-butyrate, and an ionogen and a high boiling 25 liquid intimately embodied therein, said ionogen being at least one of the materials selected from the group consisting of acids used in the formation of conductive compositions for electrolytic condensers and the stable salts thereof, and 30 said high boiling liquid being selected from the group consisting of glycerine and the glycols.

2. A spacer for dry electrolytic condensers comprising a cellulose derivative selected from the group consisting of cellulose acetate, ethyl cellulose and cellulose aceto-butyrate, and an electrolyte comprising an ionogen and a high boiling 35 liquid embodied therein, said cellulose derivative comprising a non-tacky, non-homogeneous, porous matrix carrying said electrolyte, said spacer 40 being capable of maintaining a current-blocking film on a condenser electrode during operation of the condenser with said spacer interposed between the electrodes thereof.

3. The method of making a non-tacky, non-homogeneous, porous conductive film-maintaining spacer for dry electrolytic condensers which comprises dissolving a cellulose derivative selected from the group consisting of cellulose acetate, ethyl cellulose and cellulose aceto-butyrate, at least one ionogen and at least one high 50 boiling liquid which is not a solvent for the cellulose derivative in a volatile solvent, and forming a sheet spacer therefrom by evaporating 55 said volatile solvent from a thin layer thereof.

4. The method of making a non-tacky, non-homogeneous, porous conductive film-maintaining spacer for dry electrolytic condensers which comprises dissolving the following ingredients in a common volatile solvent: (1) a cellulose derivative selected from the group consisting of cellulose acetate, ethyl cellulose and cellulose aceto-butyrate, (2) at least one ionogen selected 60 from the group consisting of acids used in the formation of conductive compositions for electrolytic condensers and the stable salts thereof and (3) at least one high boiling liquid selected 65 from the group consisting of glycerine and the glycols, and forming a sheet spacer therefrom 70 by evaporating said volatile solvent from a thin layer thereof.